

## UNITED STATES PATENT OFFICE

2,400,786

METHOD OF PREVENTING SILVERWARE  
FROM TARNISHINGJohn B. Rust, West Orange, N. J., assignor to  
Montclair Research Corporation, a corporation  
of New JerseyNo Drawing. Application April 7, 1944,  
Serial No. 530,065

5 Claims. (CL. 117—134)

This invention relates to a method of retarding the tarnishing of silver, with particular reference to retarding the surface staining of silverware.

The ready tendency for surfaces of silver to tarnish and stain on exposure to ordinary atmospheric conditions presents a constant cleaning problem which is annoying and labor-consuming. A solution of this problem would be of definite benefit not only to stores having silverware on exhibit but also to households where such silverware as candlesticks, bonbon dishes, trays, etc., are usually left exposed on tables, sideboards, etc., and consequently need frequent cleaning.

It has been suggested to protect silverware by applying a thin coating of collodion. It has also been suggested to protect silverware by confining it in a restricted spaced exposed to the vapors of a voltaile amine. While this might be accomplished under certain conditions in a store, it would be impractical in a home.

I have now found a practical solution for substantially retarding the formation of tarnish films and stain on the surfaces of silverware without any necessity whatsoever of confining the silverware to a restricted space.

It is known that guanidine and substituted guanidines may be neutralized by an aliphatic acid to give water-soluble products. I have now found that water-soluble guanidine salts of aliphatic acids exert an excellent protective action on silverware.

In practising the invention it is merely necessary to coat the silverware with a dilute solution of a water-soluble guanidine salt. A satisfactory method of accomplishing the above is to make a 1% to about 5% (preferably a 2%) solution, impregnate with this solution a wad of cotton, then rub this wad lightly over clean silverware, making certain that a film is left on every part of the surface which is to be protected. The film is then allowed to dry and given a slight buffing. The solution can also be applied by dipping or spraying. Silverware so treated will remain untarnished for periods over a month when left in ordinary atmospheric conditions while an untreated piece will be badly stained and tarnished when left under similar conditions.

Substituted guanidines suitable for use herein may be formed by heating a primary amine with guanidine (or guanidine carbonate), whereby reaction occurs with the evolution of ammonia. As primary amines for this purpose I prefer to use compounds such as ethylene diamine and

polyethylene polyamines (e. g., diethylene triamine, triethylene tetramine, tetraethylene pentamine, etc.). For use in the present invention guanidine and substituted guanidines are converted into their fatty acid salts.

As fatty acid I can use aliphatic carboxylic acids possessing ten or more carbon atoms in the molecule. Both saturated and unsaturated acids are satisfactory, such as lauric, stearic, palmitic, oleic and the fatty acids of vegetable and animal oils and fats. Considering cost and ease of use, oleic acid is suitable.

The description given in the following examples should not be construed as limiting, but only by way of illustration since those skilled in the art may make variations in the process of this invention without departing from the scope and spirit thereof.

Example 1.—One mole of stearic acid is reacted with  $\frac{1}{2}$  mole of guanidine carbonate. A 2% aqueous solution of guanidine stearate is made and applied to silverware by impregnating a cotton wad with the solution, rubbing this wad lightly over clean silverware, allowing the film to dry and giving it then a slight buffing. After application and buffing the silverware has a bright appearance and remains bright even after a month's exposure to ordinary atmospheric conditions.

Example 2.—One mole of coconut oil acids is reacted with  $\frac{1}{2}$  mole of guanidine carbonate. A 2% solution of the above reaction product is then made in a mixture of 30% of isopropanol and 68% of water. The solution is applied to silverware in the manner described in Example 1. Silverware so treated remains bright after one month.

Example 3.—One mole of oleic acid is reacted with  $\frac{1}{2}$  mole of guanidine carbonate. A 2% solution of the above reaction product is then made in a mixture of 60 parts of isopropanol and 135 parts of water. The solution is applied to silverware in the manner described in Example 1. Silverware so treated remains bright after one month.

Example 4.—One mole of stearic acid is reacted with 1 mole of diethylene triamine-guanidine (a substituted guanidine made by heating equimolecular proportions of guanidine carbonate and diethylene triamine). A 2% solution of the reaction product is then made and applied to silverware in the described manner. Silverware so treated remains bright after one month.

Example 5.—Two moles of stearic acid are reacted with 1 mole of diethylene triamine-guanidine

dine (a substituted guanidine made by heating equimolecular proportions of guanidine carbonate and diethylene triamine). A 2% solution of the reaction product is then made and applied to silverware in the described manner. Silverware so treated remains bright after one month.

I claim:

1. A process for protecting silverware from tarnishing which comprises depositing on the surface thereof a thin continuous film of a fatty acid salt of a compound selected from the group consisting of guanidine and substituted guanidines, the fatty acid containing more than 10 carbon atoms.

2. A process for protecting silverware from tarnishing which comprises applying to the surface thereof a dilute aqueous solution of a fatty acid salt of a compound selected from the group consisting of guanidine and substituted guani-

dines, removing the water therefrom and buffing the surface, the fatty acid of the salt containing more than 10 carbon atoms.

3. A process for protecting silverware from tarnishing which comprises depositing on the surface thereof a thin continuous film of guanidine stearate.

4. A process for protecting silverware from tarnishing which comprises depositing on the surface thereof a thin continuous film of guanidine oleate.

5. A process for protecting silverware from tarnishing which comprises depositing on the surface thereof a thin continuous film of the stearic acid salt of the substituted guanidine obtained by heating guanidine carbonate and diethylene triamine.

JOHN B. RUST.